

## UNITED STATES PATENT OFFICE

1,924,543

## FILAMENT

Allen B. Du Mont, Bloomfield, N. J., assignor to  
De Forest Radio Company, Jersey City, N. J.,  
a corporation of Delaware

No Drawing. Application November 26, 1928  
Serial No. 321,844

## 1 Claim. (Cl. 250—27.5)

This invention relates in general to a metal alloy particularly adapted for use in constructing filaments for electron emissive devices.

One of the objects of this invention is the provision of an alloy from which filaments for use in electron discharge devices may be constructed having desirable characteristics for such use.

Another object of this invention is the provision of filaments of this type which have a higher tensile strength than filaments of this type now known.

Another object of this invention is the provision of filaments made from the improved alloy having a high electron emissivity.

15 A further object of this invention is the production of a filament composed of a nickel chromium iron alloy.

These and other objects will appear from the following disclosure are sought by means of this 20 invention.

This invention resides substantially in the combination, construction, and proportion of parts as will be more fully disclosed hereinafter.

25 Electron discharge devices, of which the audion used in radio receiving and transmitting apparatus is an example, employ an electronically active element generally known as a cathode. These cathodes are usually provided with a coating of highly emissive substance which when 30 heated throws off electrons in large quantities. It is usual to construct these filaments of some metal such as nickel or platinum which is coated with the electron emissive substance. Filaments of nickel or platinum, however, have many disadvantages, such as extremely small cross sectional area when constructed for the correct current carrying capacities for use on voltages now common in operating radio receiving and transmitting apparatus, and as a result are very 35 fragile.

40 The filament of this invention is made of a metal alloy and is of relatively large cross sectional area when made for use in apparatus of this type and is, therefore, much more rugged, 45 having a higher tensile strength, and acts better as a cathode by reason of the larger area from which the electrons can be emitted. Furthermore, coated filaments of this nature are found to have an electron emissivity which is three 50 times greater than the emissivity of thoriated tungsten filament. In addition, by reason of its relatively greater size the filament is operated at a much lower temperature and, in fact, at a very dull red heat so as to be hardly visible. The 55 result is that devices of this nature are not called

upon to dissipate as much heat as they would when employing a tungsten filament which is easily heated to a white hot incandescence. The absence of this excess heat produces better operating characteristics.

60 The filament is constructed of a metal alloy comprising nickel, chromium and iron. In the best practice the proportions are chromium 15%, iron 20%, and nickel 65%. A metal alloy of 65 nickel, iron and chromium in these percentages produces a filament having the characteristics pointed out above. It has been found that with a filament constructed with the above proportions of ingredients, the filament will exhibit 70 amply effective emission at low temperatures, for instance when the filament is at an almost imperceptible red. The emission of this type of filament is approximately sixty times that of ordinary thoriated tungsten filament at the same 75 temperature. In one type of filament constructed in accordance with the invention the filament was in the form of a heavy ribbon and operated at 750 degrees centigrade as contrasted with 2300 degrees centigrade for the usual thoriated tungsten filament. At 3 volts this filament gives about 80 the same emission as the usual thoriated tungsten filament at full 5 volts, while the life of this filament is several times as great as that of a corresponding thoriated tungsten filament.

85 It is, of course, to be understood that good results can be secured in accordance with this invention by varying the proportions given and I do not, therefore, desire to be structurally limited to the exact proportions given but to a range 90 of equivalent proportions which produce a filament of substantially the same characteristics.

95 What I seek to secure by United States Letters Patent is:

A filament for electron discharge devices comprising a metal alloy consisting of approximately 15% chromium, iron 20%, and approximately 65% nickel, whereby the filament may be effectively operated as an emitter at a dull red heat, and a coating of electron emissive material on 100 said filament.

ALLEN B. DU MONT.

105

110